

J. ABSTERDAM.

## Introducing Gas Fuel into a Converter for Making Steel, &c.

No. 84,336.

Patented Nov. 24, 1868.



Witnesses  
Eunice F. Kadenbush  
Chas Wahler

Everett  
John Rotterdam  
Law Santwood & Co.  
Atty.

# United States Patent Office.

JOHN ABSTERDAM, OF NEW YORK, N. Y.

Letters Patent No. 84,336, dated November 24, 1863.

## IMPROVED PROCESS FOR INTRODUCING GAS-FUEL INTO A CONVERTER FOR MAKING STEEL AND REFINING IRON.

The Schedule referred to in these Letters Patent and making part of the same.

To all whom it may concern:

Be it known that I, JOHN ABSTERDAM, of the city, county, and State of New York, have invented a new and improved Process for Introducing Fuel into a Converter for Making Steel and Refining Iron; and I do hereby declare the following to be a full, clear, and exact description thereof, which will enable those skilled in the art to make and use the same.

This invention consists in introducing fuel, either in a gaseous or solid form, into the molten metal in the converter, by suction, in contradistinction to the process heretofore known, where fuel has been introduced into the molten metal by force.

In order to facilitate the explanation of my process, I will refer to the annexed sketch, which represents a sectional view of an apparatus such as I may use in carrying out my invention, though I will here remark that I do not wish to confine myself to any particular apparatus, but reserve the right to make such changes in the same as may be desirable, according to varying circumstances.

In carrying out my process, I introduce the iron to be refined, or to be converted into steel, in a molten state, in a converter, A, which is provided with a series of openings, *a*, in its bottom, and the neck of which connects with an exhaust-apparatus, B, of any suitable construction. The openings, *a*, are closed by plugs, until the molten metal has been introduced, and the exhausting-apparatus has been started. Then the plugs are removed, and a current of air is made to pass through the molten metal by suction, as fully described in Letters Patent granted to me, January 23, 1866. As the air passes through the molten metal, it burns away the carbon contained in the iron, dilating the impurities contained therein, which are extracted from the molten mass by suction, and the iron is refined; but if the process is carried on a little too long, or if it is desired to convert the iron into steel, it is necessary to introduce a fresh supply of fuel to the action of the streams of air in the molten metal, so as to prevent a too rapid decarbonization of the molten cast-iron, in order to better deprive the metal of its impurities.

The materials which I generally introduce through the molten iron, during the process of conversion, to produce fuel, are carbonaceous gases, or ground or powdered solid carbonaceous substances.

The solid substances above mentioned are introduced through openings, *a\**, in the sides of the converter, by connecting said openings with suitable hoppers.

By the suction of the air, the powdered materials are carried into and through the molten metal in the converter.

The gaseous materials are introduced by means of a pipe, *b*, which is situated under the converter, and connects with a chamber, *c*, from the top of which extends a series of nipples, *d*, which correspond in number and position to the holes, *a*, in the bottom of the converter. If gas is admitted through the pipe *b*, it issues from the nipples *d*, and the suction of the air carries the same into the converter.

If a hydrocarbon-liquid, such as crude petroleum, is admitted to the chamber *c*, it may be desirable to provide the nipples *d* with small wick-tubes, so that the

liquid will be raised by capillary attraction, and that, by burning said liquid as it rises in the nipples, a flame is produced which contains a large quantity of free carbon, and which is carried into the converter by the suction of the air.

The chamber *c* will be so arranged that it can be raised or lowered by means of a foot-lever or otherwise, so that its position in relation to the converter can be adjusted. It may also be provided with plugs fitting over the nipples, so that, by raising said chamber, all the holes *a*, in the bottom of the converter, can be stopped up simultaneously.

By introducing fuel into the converter by suction, I gain the following principal advantages: I require no distinct apparatus for forcing in the fuel, the fuel being carried in spontaneously by suction with the current of air; the quantity of fuel introduced can be regulated with the greatest nicety, and the process of refining iron or making steel is thereby materially facilitated; and, finally, I can regulate the introduction of the quantity of fuel and air necessary to produce the greatest amount of heat required for refining the iron or converting it into steel, it being very well known that cast-iron contains only a small percentage of carbon, which, if used as the only fuel for producing the combustion required to purify the molten metal, I find that said carbon is burned away before the process of refining or purifying is finished; that is to say, the iron becomes decarbonized before the metal is perfectly freed from its impurities.

But by letting an additional amount of fuel, as required, enter with the air, through the molten mass, by suction, I produce a very intense heat, and at the same time the requisite amount of combustible matter is furnished to the oxygen of the air therein, which prevents a too rapid decarbonization of the metal in the converter.

This operation will be readily understood, because, so long as I supply carbon to the oxygen of the streams of air passing through the molten metal, I also continue the heat in the converter, without burning all or too much of the carbon of the iron before the metal is deprived of its impurities, in contradistinction to the well-known Bessemer process of converting cast-iron into steel, which is carried on "without the use of fuel for heating or continuing to heat the crude molten metal." (See his claim of November 11, 1856.) In this case, the carbon of the iron is burned out, and the metal becomes red hot, whether the metal in the converter is deprived of its impurities or not; whereas, by the introduction of fuel in the manner above described in my process, I have complete control of the purification and conversion of the metal in the converter.

Having thus described my invention,

What I claim as new, and desire to secure by Letters Patent, is—

The process, herein described, of introducing fuel into the molten metal in a converter, by suction.

JOHN ABSTERDAM.

Witnesses:

W. HAUFF,

CHAS. WAHLERS.